

1,148,381.

J. F. HASKINS.  
NON-OFFSET SURFACE COVERING FOR IMPRESSION CYLINDERS.  
APPLICATION FILED APR. 23, 1915.

Patented July 27, 1915.

Fig. 1.



Fig. 2.



WITNESSES:

Edw. Thorpe  
John Bader

INVENTOR  
J. F. Haskins.

BY *M. M. Co.*  
ATTORNEY

# UNITED STATES PATENT OFFICE.

JOHN F. HASKINS, OF NEW YORK, N. Y.

## NON-OFFSET SURFACE-COVERING FOR IMPRESSION-CYLINDERS.

1,148,381.

Specification of Letters Patent. Patented July 27, 1915.

Application filed April 23, 1915. Serial No. 28,273.

To all whom it may concern:

Be it known that I, JOHN F. HASKINS, a citizen of the United States, and a resident of the city of New York, borough of Manhattan, in the county and State of New York, have invented a new and Improved Non-Offset Surface-Covering for Impression-Cylinders, of which the following is a full, clear, and exact description.

10 This invention relates to the cylinders of printing presses and has particular reference to the surface coverings for the impression or offset cylinders of such machines.

15 Among the objects of the invention is to provide a surface covering for an impression or packing cylinder of such nature or character as to obviate the use of the troublesome and expensive tympan sheet so commonly used for receiving and absorbing the 20 surplus oil, ink or smut from the printed sheet.

Another object of the invention is to provide a surface covering for the impression cylinder of a printing press, the same having the properties necessary to insure long 25 and severe use without renewal or change.

Another object of this invention is to provide a composition of matter adapted to be applied to any fabric or flexible body for 30 use upon an impression cylinder of a web printing press, said composition of matter constituting a distinct commercial commodity and serving, when applied as stated, to render the blanket or other cylinder covering 35 non-offset in nature and of a character adapted to counteract the effect of accumulations of static electricity.

The foregoing and other objects of the invention will hereinafter be more fully described and claimed and illustrated in the drawings forming a part of this specification in which like characters of reference indicate corresponding parts in both the views, and in which—

45 Figure 1 is a plan view of a section of a blanket indicating the relation and number of plies or layers constituting the same, a corner of each ply being turned over or exposed to plainly indicate the relation of 50 these parts; and Fig. 2 is a longitudinal section of the same on the line 2—2 of Fig. 1.

In carrying out this invention it is obvious that in the manufacture of blankets I 55 do not wish to be limited to any particular fabric or body construction. Said body or blanket may be of a plurality of plies or

layers, the fibers of the layers being arranged at an angle to one another or they may be arranged rectangularly or otherwise, and secured together by any suitable adhesive material with or without the use of an intermediate textile fabric.

As a practical embodiment of the invention, as carried out by practical experiments, I construct a blanket of laminated form 60 having two plies 10 of tough, strong, flexible non-elastic fabrics of considerable body or thickness. Between such two plies I sandwich a strip or layer of adhesive material carried preferably upon a textile 65 fabric or layer 11 which serves to unite the inner and adjacent surfaces of the two outer plies firmly and permanently together or to the innermost ply 11. Either or both, preferably both, of the outer surfaces of the 70 two main plies 10 above described are then coated and impregnated with a surface coating 12 of some suitable mixture or compound of a non-oxidizing nature made preferably of animal and vegetable viscous 75 ingredients and possessing a number of important properties in the printing press art. Each coating or covering 12 constitutes a distinct ply of the blanket, adding appreciably to the micrometer thickness thereof, as 80 well as being thoroughly and permanently incorporated and impregnated in and with the main plies 10. As an illustration of a suitable compound for treating or coating the blanket, I prefer to employ a chemically 85 neutralized composition of gelatin, kept in soft condition by the addition of glycerin, and rubber, with an overlying japan, made from an alcohol solvent, copal gum and another vegetable gum such as rubber and a 90 small percentage of glycerin.

By way of a more definite specification of the ingredients of the composition of matter employed in carrying out this invention, but without unnecessarily limiting myself to the 100 exact proportions, I may explain that as the main or first coating I employ a chemically neutralized gelatin in connection with glycerin and water in substantially the proportions of four pounds of gelatin, one-half 105 pound of glycerin, and eight pounds of water. The gelatin and the glycerin are mixed and dissolved in the water, and to the mixture or solution I add about two pounds of a solution of rubber or what may be 110 better termed a rubber varnish made from india rubber, turpentine, benzin, blown lin-

seed oil, and lampblack, in the proportions by weight of substantially ten parts india rubber, ten parts turpentine, twenty parts benzin, forty-five parts linseed oil, five parts lamp-black. This rubber varnish is preferably made by dissolving and mixing by agitation and friction the india rubber, turpentine and benzin, and to such completed mixture are added the linseed oil and lampblack, stirring very thoroughly. A second or japan coating is then applied, said coating being composed of copal gum, alcohol, glycerin, and rubber varnish made as described above. The relative proportions of these parts for making the japan coating are substantially by weight as follows: copal gum, twenty parts; alcohol, one hundred parts; glycerin, one part, and rubber varnish, one part.

20 Among the primary virtues of this surface coating 12 is that it has proved in practice to be absolutely non-offset or ink- and oil-resisting, whereby there is no deposit made upon it from the printed sheet while receiving the second impression. Thereby I am able to produce a perfectly clear and satisfactory printing effect, without the use of a tympan sheet of muslin or other fabric which is so commonly used. In fact, my printing result is clearer and better than when the tympan sheet is used.

25 The surface coating 12 above referred to is of a pronounced wear-sustaining nature, it having proved capable of sustaining from three to five million impressions without change and without requiring to be renewed. The actual wear is found not to exceed more than two one-thousandths of an inch as indicated by micrometer caliper to each million impressions, thereby making it possible to maintain nearly perfect unit peripheral relation of plate and impression cylinders and to hold to nearly true pitch line the relation of the gears.

30 As is well recognized in the operation of large cylinder presses, much difficulty is encountered as a result of static electricity in cold snappy weather, thus the tension which must be maintained under ordinary circumstances upon the paper to hold a smooth pulling web and a proper head margin cut-off is unnecessarily great, resulting frequently in the parting of the paper if the pull thereon is sufficient to prevent the wrinkling of the paper and bad margin cut-off due to the electrical influences common to the usual blanket constructions. In accordance with this invention however, due

largely to the glycerin used in compounding the material constituting the coating 12, no 60 artificial humidity or heat is required to combat the accumulations of static electricity, and hence the machine and paper may be operated uniformly smoothly at all times.

65 I am aware that numerous propositions have been made as improvements in printing press blankets, some of which claim to be of an oil- and ink-proof nature, but, in my vast experience as a printing press expert, 70 I believe I am the first to devise a printing press blanket or a surface coating for a printing press blanket or packing which has the property, not only of being a non-absorbent of ink and oil, but one which actually 75 resists the reception of the surplus ink, oil or smut from the printed sheet passing over the impression cylinder coated with my improvement.

I claim:

80 1. The herein described non-offset surface covering for printing press blankets, the same comprising a composition of matter including a chemically neutralized composition of gelatin, kept in soft condition by the addition of glycerin, and rubber, with an overlying japan made from an alcohol solvent, copal gum and another vegetable gum and a small percentage of glycerin.

2. The herein described coating for a 90 printing press blanket, the same comprising a mixture of chemically neutralized gelatin, glycerin and rubber, and an overlying surface coating comprising vegetable gums in solution and including a small portion of 95 glycerin.

3. The herein described coating material for printing press blankets, the same comprising a main body coating including a mixture of glycerin and rubber, and a surface coating therefor of ink-resisting wear-sustaining properties including an alcohol solvent, copal gum.

4. In a surface covering for printing press blankets, the combination of a chemically 105 neutralized composition of gelatin, an oil, and rubber, constituting a plastic body adapted to impregnate the blanket to which it is applied, and a surface coating therefor of an ink-resisting wear-sustaining nature 110 comprising a solution of vegetable gums and a small percentage of glycerin.

JOHN F. HASKINS.

Witnesses:

GEO. L. BEELER,  
PHILIP D. ROLLHAUS.